

R. V. MATTISON, JR.  
INTEGRAL LOCOMOTIVE MATTRESS.  
APPLICATION FILED AUG. 19, 1907.

912,971.

Patented Feb. 16, 1909.



WITNESSES:

John C. Bergner  
Wm. J. Spel.

INVENTOR:

RICHARD V. MATTISON JR.,

By Tracy & Paul  
attorneys

# UNITED STATES PATENT OFFICE.

RICHARD V. MATTISON, JR., OF UPPER DUBLIN TOWNSHIP, MONTGOMERY COUNTY, PENNSYLVANIA, ASSIGNOR TO KEASBEY & MATTISON COMPANY, OF AMBLER, PENNSYLVANIA, A CORPORATION OF PENNSYLVANIA.

## INTEGRAL LOCOMOTIVE-MATTRESS.

No. 912,971.

Specification of Letters Patent. Patented Feb. 16, 1909.

Application filed August 19, 1907. Serial No. 389,114.

*To all whom it may concern:*

Be it known that I, RICHARD V. MATTISON, Jr., of Upper Dublin township, in the county of Montgomery and State of Pennsylvania, have invented certain new and useful Improvements in Integral Locomotive-Mattresses, whereof the following is a specification, reference being had to the accompanying drawings.

10 My improvements relate to a non-heat conducting and incombustible mattress formed entirely of mineral ingredients and so formed, constructed and arranged as to be adapted as an integral structure to be inserted between the boiler of a locomotive engine and its jacket. The advantage of having a heat insulating substance, which is thus customarily inserted between the boiler and jacket formed as an integral structure, 15 is that when the locomotive is under repairs the removal and replacement of the insulating means is rendered much more easy. All this is accomplished without substantial loss to the efficiency of the heat insulating means.

In the accompanying drawings, Figure I represents a view in side elevation of a locomotive boiler to which my improvements have been applied, the portion of the mattress between the broken lines X, X, being indicated as removed in order to show a longitudinal section of the mattress at the region between the broken lines. Fig. II, represents a transverse section through the 30 same on the line II, II, of Fig. I, looking in the direction of the arrows. Fig. III, represents a transverse section through the same on the line III, III, of Fig. I, looking in the direction of the arrows. Fig. IV, is 35 a view in elevation of the rear end of the boiler, which is at the right hand side in Fig. I. Fig. V, is a detailed fragmentary sectional view showing the internal construction of the mattress.

40 The mattress is formed as a single integral structure properly cut and shaped to be placed over and around the entire portion of the boiler which is to be insulated and covered by its jacket. For this purpose it is shaped as follows:—The sheets 1, 2, 3, and 4, are formed of sufficient length and width to properly surround the respective portions of the boiler corresponding thereto. These sheets are provided with openings,

which fit around lugs or brackets upon the 55 side of the boiler used for supporting purposes. Sheet 2, is provided with an opening for the reception of the steam dome 10. Sheet 4, is provided with openings for the reception of various pipes and mechanism 60 on the top of the boiler within the cab. The back head of the boiler or fire box face is covered with a sheet 16, also united to the remainder of the mattress in any suitable manner. This sheet is provided with numerous openings for the reception of the 65 throttle valve, steam gages, and so forth, as clearly seen in Fig. IV.

The various sheets are quilted at intervals as indicated at 20, in Fig. V. The mattress is maintained in position upon the boiler by means of asbestos tape or metallic bands 22, as clearly indicated in Fig. I. Upon the sheet 2, is secured the tube 9, which fits around the steam dome 10, and is secured 75 in position by means of asbestos tape or metallic bands 24.

The entire structure consists of two layers 14, 15, of an asbestos textile fabric with a plurality of layers 17, 18, 19, of asbestos fiber felt interposed, the whole being formed 80 into a mattress by sewing the edges 25 and 26 of the textile fabrics together and by quilting at intervals.

The textile fabric may be of the ordinary 85 woven asbestos cloth, but for the sake of strength and permanency I prefer to employ a reinforced wire cloth, in which fine steel or other metallic wire is woven along with the asbestos thread.

90 The interior of the structure is formed of a plurality of layers of asbestos fiber felt. This is a homogeneous mass of fibrous asbestos sufficiently cemented together by silicate of soda, or plaster of paris to enable it 95 to maintain its shape, but not to the exclusion of a large amount of air, filling the interstices between the asbestos fibers. Asbestos fiber felt is usually furnished in sheets about three feet wide, and of indefinite 100 length, and for the purpose of preparing my mattress I preferably employ three layers of this fiber felt arranging the strips in adjacent layers, so as to run at right angles and break joints. By thus employing asbestos 105 fiber felt instead of loose or flocculent asbestos for the interior packing of the mattress, I prevent the jarring motion of the

locomotive from shaking the asbestos fiber down to the edges of the mattress along the side to the detriment of the non-heat conducting qualities of the upper portion of the mattress.

By making the packing three-ply I increase the amount of imprisoned air space. The asbestos fiber felt sheets are ordinarily about three-eighths of an inch in thickness, so that three of them when quilted together, produce a mattress of about one inch in thickness.

Having thus described my invention, I claim:—

15 1. An asbestos locomotive mattress consisting of outer layers of asbestos textile fabric and a plurality of inner layers of sheets of asbestos fiber felt, each sheet of fiber felt consisting of a homogeneous mass of fibrous asbestos sufficiently cemented together to enable it to maintain its shape, yet retain a considerable amount of air in its

interstices, the textile covering being united at its edges and the whole being further united by quilting.

2. An asbestos locomotive mattress consisting of outer layers of asbestos textile fabric and a plurality of inner layers of sheets of asbestos fiber felt, each sheet of fiber felt consisting of a homogeneous mass of fibrous asbestos sufficiently cemented together by silicate of soda, or plaster of paris, to enable it to maintain its shape, yet retain a considerable amount of air in its interstices, the textile covering being united at its edges and the whole being further united by quilting.

In testimony whereof, I have hereunto signed my name, at Philadelphia, Pennsylvania, this fifth day of August, 1907.

RICHARD V. MATTISON, JR.

Witnesses:

JAMES H. BELL,  
E. L. FULLERTON.